

# UNITED STATES PATENT OFFICE.

ARON HAMBURGER, OF LONDON, ENGLAND.

## COLOR PHOTOGRAPHY.

1,059,867.

Specification of Letters Patent.

Patented Apr. 22, 1913.

No Drawing.

Application filed May 27, 1912. Serial No. 700,051.

*To all whom it may concern:*

Be it known that I, ARON HAMBURGER, a citizen of the United States of America, and residing at 38 Dover street, London, 5 W., England, have invented certain new and useful Improvements in and Relating to Color Photography, of which the following is a specification.

This invention relates to the obtaining of 10 color prints of photographs.

This invention has for its object to provide improved processes for the production of a yellow tone in prints of photographs and to provide a method of producing color 15 photographs which will substantially simplify the methods heretofore proposed.

The invention consists in a process for obtaining a yellow tone in prints of photographs consisting in bleaching an image obtained on a silver chlorobromid or other suitable light sensitive medium to any desired extent and toning the bleached image by the action of a suitable mercuric iodid solution.

25 This invention also consists in a process of obtaining color photographs in which a print is obtained on a silver chlorobromid or other suitable light sensitive medium from the negative corresponding to the yellow color, is then bleached to any desired extent and then toned by the action of potassium mercuric iodid or alkali mercuric iodid & g. by the action of a solution obtained by mixing solutions of mercuric chlorid and potassium iodid, whereby a yellow color print can be obtained having a key or foundation of practically panchromatic gray.

30 This invention further consists in a yellow color print the yellow tone of which is due to a mercury-silver iodid.

This invention further consists in a color print of a color photograph having a key or foundation of practically panchromatic 35 gray.

The invention is based on the discovery that if a silver print be bleached by a suitable bleaching solution such as potassium bromid and potassium ferricyanid and then 40 developed or toned with a solution obtained by mixing mercuric chlorid and potassium iodid solutions in suitable proportions a yellow print of good quality is obtained. Further if the print so treated be one obtained 45 from the negative corresponding to the yellow of a three color photograph the result-

ant photograph is of particular brilliance and accuracy in color reproduction. This is apparently due to the fact that the print obtained from the negative corresponding to the yellow color is more or less panchromatic and that the yellow toning method above described produces the yellow tone irrespective of the faint practically panchromatic gray image which remains as a 60 key or foundation to the print. When red and blue prints obtained by any suitable method from red and blue printing negatives are superposed upon this yellow gray key, the resultant color photograph is therefore apparently a four color photograph 65 obtained without the necessity of specially producing a panchromatic gray and by utilizing this feature the production of color prints is considerably simplified. Although 70 even if the print be quite bleached out the more or less panchromatic gray is to some extent redeveloped on toning it is preferable only to carry the bleaching sufficiently far to leave a faint gray image the extent 75 of bleaching varying of course with each 80 particular subject.

In explanation of the term "panchromatic" used in the specification to modify "gray", it should be said that in the making of three-color photographs a set of 85 three negatives is commonly made of the object to be photographed, each through a separate color filter, corresponding to the desired three colors. The filter used for the 90 yellow is imperfect in its action in filtering the light rays, and accordingly the print obtained from the negative corresponding to the yellow color of the object is composed not only of an image corresponding to the 95 yellow components, but also contains an image of less intensity formed from rays corresponding to the other color components of the object photographed. When such a print is bleached in the 100 manner described above the main bulk of the image on the print, corresponding to the yellow color of the object photographed, disappears, and leaves the faint gray image, which is the panchromatic 105 image above referred to, that is, one formed by all the color components of the object in their true values. In the next step of my process, of toning, as described, this gray image is apparently unaffected. Accordingly, when the yellow print thus formed is 110 combined with the corresponding red and

blue prints, made in any suitable manner, the resultant color photograph is formed with an underlying faint gray key or image. This key results, when the three color prints 5 are assembled, as stated, in effecting a certain compensation for the necessary inaccuracies of the process of negative-making, with the result that in the resultant color photograph remarkably fine effects and accurate reproduction of colors are produced.

10 In carrying out the process in obtaining color prints for color photographs in one form a bromid or chlorobromid print is first obtained from the negative corresponding to the yellow. It is desirable that the paper of the print should be parchmentized or have been otherwise suitably treated to prevent shrinkage. This print is then bleached in either of the following solutions 15 according to whether a pure yellow or reddish yellow is desired. 1 part of 5% potassium ferricyanid solution. 1 part of 5% potassium bromid solution, or 30 parts of 5% lead nitrate solution. 10 parts of 10% potassium ferricyanid solution. 10 parts of 20 10% aluminium nitrate. 1 part of nitric acid. 15 parts of acetic acid. 50 parts of water.

25 The bleaching is carried out until a faint gray image only remains when after washing as usual the print is immersed in the following toning solution:—40 parts of 6% mercuric chlorid solution. 60 parts of 8% potassium iodid solution.

30 When the desired tone is attained the prints are removed and washed in the usual way. It is to be observed that the tone continues to develop after completion of the immersion in the toning bath and allowance 35 must be made for this in determining the time of withdrawal. The formation of yellow can be arrested by immersing the print in an acid bath at any time during the toning. In this way a print is obtained 40 in a fine yellow color which corresponds to the yellow portion of the picture being produced and which possesses a key or foundation of practically panchromatic gray. This has been obtained in one operation without 45 any special skill and avoids the need of registration or fixing necessary where a separately produced panchromatic key or foundation is employed as has been proposed. The print so obtained can now in 50 any suitable way be combined with the remaining color prints which may be of any suitable kind.

55 It will be understood that the present invention may be applied to prints on transparent or translucent media as well as to prints on an opaque base.

60 The print which is treated may be one obtained on a bromid, chloro-bromid or other silver or suitable salt containing light 65 sensitive medium and the bleaching solution

may be of any suitable kind, *e. g.* it may be a chromic acid or bichromate bleaching solution.

It is to be understood that the methods of obtaining the mercury silver iodid image 70 and of obtaining the print with a gray key or foundation above described are referred to by way of example only and may be considerably varied without departing from the spirit of the present invention.

75 Having now described my invention what I claim as new and desire to secure by Letters Patent is:—

1. A process for obtaining a colored photographic print suitable for combination with prints of other colors to form a resultant color photograph, consisting in making a negative of the object to be reproduced through a yellow filter, making a print therefrom on a silver-containing light-sensitive medium, bleaching the print until only a faint gray image remains, washing, toning in a suitable mercuric iodid solution, until a yellow tone is obtained, removing from the solution and washing, substantially as described.

80 2. A process for obtaining a colored photographic print suitable for combination with prints of other colors to form a resultant color photograph, consisting in making a negative of the object to be reproduced through a yellow filter, making a print therefrom on a silver-containing light-sensitive medium, bleaching the image to any desired extent, and toning the bleached image 85 in a solution obtained by mixing solutions of mercuric chlorid and potassium iodid until a yellow tone is obtained, and removing from the solution and washing, substantially as described.

90 3. A process for obtaining a colored photographic print suitable for combination with prints of other colors to form a resultant color photograph, consisting in making a negative of the object to be reproduced 95 through a yellow filter, making a print therefrom on a silver-containing light-sensitive medium, bleaching the image to any desired extent in a solution of potassium bromid and potassium ferri-cyanid and 100 toning the bleached image in a suitable mercuric iodid solution until a yellow tone is obtained and removing from the solution and washing, substantially as described.

105 4. A process for obtaining a colored photographic print suitable for combination with prints of other colors to form a resultant color photograph, consisting in making a print on a silver-containing light-sensitive medium, bleaching the same until only a 110 faint gray image remains, and toning the bleached image in a suitable mercuric iodid solution until a yellow tone is obtained and removing from the solution and washing, substantially as described.

115 5. A process for obtaining a colored photographic print suitable for combination with prints of other colors to form a resultant color photograph, consisting in making a print on a silver-containing light-sensitive medium, bleaching the same until only a 120 faint gray image remains, and toning the bleached image in a suitable mercuric iodid solution until a yellow tone is obtained and removing from the solution and washing, substantially as described.

5. A process for obtaining a colored photographic print suitable for combination with prints of other colors to form a resultant color photograph, consisting in making a negative of the object to be reproduced through a yellow filter, making a print therefrom on a silver-containing-light sensitive-medium, bleaching the image to any desired extent and toning the bleached image in a suitable mercuric iodid solution until the desired yellow tone is obtained, removing the print from the solution, immersing in an acid bath to arrest further formation of the yellow color and washing, substantially as described. 10
6. A process for obtaining a colored photographic print suitable for combination with prints of other colors to form a resultant color photograph, consisting in making a print on a silver-containing-light-sensitive medium from a negative of the yellow portion of the object to be reproduced, bleaching the print until only a faint gray image remains, washing and toning in a solution formed by mixing together approximately 40 parts of substantially 6 per cent. mercuric chlorid solution and 60 parts of substantially 8 per cent. potassium iodid solution, and removing from the solution 15
- when a yellow tone has developed and washing, substantially as described. 30
7. As a new article of manufacture, a yellow color print having a key or foundation of gray, the yellow tone of which print is due to a mercury silver-iodid, substantially as described. 35
8. As a new article of manufacture, a photographic color print having yellow elements representing selectively the yellow components only of the object photographed, which yellow elements are caused by iodids of mercury and silver, substantially as described. 40
9. As a new article of manufacture, a photographic color print of a permanently bright yellow corresponding selectively to the yellow components only of the object photographed and due to a mercury silver iodid, the said print having a key or foundation of practically panchromatic gray, substantially as described. 45

This specification signed and witnessed this 17th day of May 1912.

ARON HAMBURGER.

Witnesses:

D. J. JOHNSTON,  
G. E. HOSKINS.